



US011124851B2

(12) **United States Patent**  
**Mao et al.**

(10) **Patent No.:** **US 11,124,851 B2**  
(45) **Date of Patent:** **\*Sep. 21, 2021**

(54) **1900 MPA GRADE PRESS HARDENING STEEL BY THIN SLAB CASTING AND DIRECTLY ROLLING AND METHOD FOR PRODUCING THE SAME**

(71) Applicant: **WUHAN IRON AND STEEL COMPANY LIMITED**, Hubei (CN)

(72) Inventors: **Xinping Mao**, Hubei (CN); **Libo Pan**, Hubei (CN); **Kuanhui Hu**, Hubei (CN); **Shuize Wang**, Hubei (CN); **Rui Ge**, Hubei (CN); **Lijun Li**, Hubei (CN); **Tao Peng**, Hubei (CN); **Xiaoping Duan**, Hubei (CN); **Fang Fang**, Hubei (CN)

(73) Assignee: **WUHAN IRON AND STEEL COMPANY LIMITED**, Hubei (CN)

(\*) Notice: Subject to any disclaimer, the term of this patent is extended or adjusted under 35 U.S.C. 154(b) by 315 days.

This patent is subject to a terminal disclaimer.

(21) Appl. No.: **16/322,108**

(22) PCT Filed: **Aug. 1, 2017**

(86) PCT No.: **PCT/CN2017/095492**

§ 371 (c)(1),  
(2) Date: **Jan. 31, 2019**

(87) PCT Pub. No.: **WO2018/036346**

PCT Pub. Date: **Mar. 1, 2018**

(65) **Prior Publication Data**

US 2019/0185953 A1 Jun. 20, 2019

(30) **Foreign Application Priority Data**

Aug. 24, 2016 (CN) ..... 201610713630.2

(51) **Int. Cl.**  
**C21D 8/02** (2006.01)  
**C22C 38/06** (2006.01)

(Continued)

(52) **U.S. Cl.**  
CPC ..... **C21D 8/0263** (2013.01); **C22C 38/001** (2013.01); **C22C 38/02** (2013.01);  
(Continued)

(58) **Field of Classification Search**  
CPC ..... B21B 1/46; B22D 11/001; C21D 1/18;  
C21D 8/0205; C21D 8/0231; C21D  
8/0263; C22C 33/04; C22C 38/18; C22C  
38/32  
(Continued)

(56) **References Cited**

**U.S. PATENT DOCUMENTS**

3,269,007 A \* 8/1966 O'Donnell ..... B21D 1/02  
72/178  
4,531,973 A \* 7/1985 Nixon ..... C21B 13/12  
75/10.41  
(Continued)

**FOREIGN PATENT DOCUMENTS**

CN 101586208 11/2009  
CN 102031456 A \* 4/2011  
(Continued)

**OTHER PUBLICATIONS**

NPL: on-line English translation of CN-105518173-A, Apr. 2016  
(Year: 2016).\*

(Continued)

*Primary Examiner* — Jie Yang

(74) *Attorney, Agent, or Firm* — JCIP Global Inc.

(57) **ABSTRACT**

A press hardening steel by a thin slab and having a tensile strength of 1900 MPa or more includes following components by weight: C: 0.31-0.40%, Si: 0.36-0.44%, Mn: 1.6-

(Continued)



2.0%, P≤0.006%, S≤0.004%, Als: 0.015-0.060%, Cr: 0.36-0.49%, Ti: 0.036-0.045% or Nb: 0.036-0.045% or V: 0.036-0.045% or a mixture of any two or more of the above in any proportion, B: 0.004-0.005%, Mo: 0.26-0.35%, and N≤0.005%. A method for producing the press hardening steel includes following steps: molten iron desulphurization; smelting and refining by an electric furnace or converter; continuous casting; descaling treatment before entering a soaking furnace; heating and soaking; high pressure water descaling before entering a rolling mill; hot rolling; cooling; coiling; austenitizing; die deforming and quenching.

## 2 Claims, 1 Drawing Sheet

### (51) Int. Cl.

*C22C 38/00* (2006.01)  
*C22C 38/02* (2006.01)  
*C22C 38/22* (2006.01)  
*C22C 38/24* (2006.01)  
*C22C 38/26* (2006.01)  
*C22C 38/28* (2006.01)  
*C22C 38/32* (2006.01)  
*C22C 38/38* (2006.01)  
*C21D 1/18* (2006.01)

### (52) U.S. Cl.

CPC ..... *C22C 38/06* (2013.01); *C22C 38/22* (2013.01); *C22C 38/24* (2013.01); *C22C 38/26* (2013.01); *C22C 38/28* (2013.01); *C22C 38/32*

(2013.01); *C22C 38/38* (2013.01); *C21D 1/18* (2013.01); *C21D 8/0205* (2013.01); *C21D 8/0231* (2013.01); *C21D 2211/008* (2013.01)

### (58) Field of Classification Search

USPC ..... 148/330  
 See application file for complete search history.

### (56) References Cited

#### U.S. PATENT DOCUMENTS

2019/0177811 A1\* 6/2019 Mao ..... C21D 8/021  
 2019/0185952 A1\* 6/2019 Mao ..... C22C 38/18

#### FOREIGN PATENT DOCUMENTS

|    |               |                        |
|----|---------------|------------------------|
| CN | 102296242     | 12/2011                |
| CN | 102965573     | 3/2013                 |
| CN | 103320702     | 9/2013                 |
| CN | 103658178     | 3/2014                 |
| CN | 105518173 A * | 4/2016 ..... C21D 9/48 |
| CN | 106086684     | 11/2016                |

#### OTHER PUBLICATIONS

NPL: on-line English translation of CN-102031456-A, Apr. 2011 (Year: 2011).\*

“International Search Report (Form PCT/ISA/210)”, dated Nov. 10, 2017, with English translation thereof, pp. 1-4.

\* cited by examiner



**1900 MPa GRADE PRESS HARDENING  
STEEL BY THIN SLAB CASTING AND  
DIRECTLY ROLLING AND METHOD FOR  
PRODUCING THE SAME**

**CROSS-REFERENCE TO RELATED  
APPLICATION**

This is a 371 application of the International PCT application serial no. PCT/CN2017/095492, filed on Aug. 1, 2017, which claims the priority benefits of China Application No. 201610713630.2, filed on Aug. 24, 2016. The entirety of each of the above-mentioned patent applications is hereby incorporated by reference herein and made a part of this specification.

**BACKGROUND OF THE INVENTION**

**1. Technical Field**

The present invention relates to a steel for automobile parts and a producing method thereof, and in particular, to a press hardening steel by thin slab casting and direct rolling and having a tensile strength of 1900 MPa or more and a production method thereof. The producing method is adapted for a product having a thickness range of 0.8 to 2 mm.

**2. Background**

With the development of automobile industry and the gradual development of automobile design and manufacturing in a direction of energy conservation, environmental protection and safety in the automobile industry, lightweight automobile designs have become the tendency of automobile design for a long time now and in future.

The researches show that there was a linear relationship between an overall weight and energy consumption of an automobile. According to statistics, fuel efficiency can be increased by 6% to 8% for every 10% reduction in automobile weight. One of the most important ways to reduce the weight of an automobile is to use a high-strength and ultra-high-strength steel, so that a curb weight of the automobile can be greatly reduced without compromising a collision safety and the comfort. However, as the strength continues to increase, formability of a steel sheet will become worse, especially for an ultra-high-strength steel of above 1900 MPa. During the forming process, there will be problems such as cracking, springback and low dimensional accuracy of parts. Furthermore, higher requirements are imposed on stamping equipment, that is, a large-tonnage stamping machine and a high-wearing die are required, and a life cycle of the die is greatly affected. At present, there is no cold forming stamping equipment and die capable of forming 1900 MPa or above in the country.

At present, a tensile strength of existing press hardening steel in the country and abroad cannot reach 1900 MPa or more, and all of them are cold-rolled annealed or pre-coated after being cold-rolled annealed. The production processes include: metal desulphurization→converter steelmaking→external refining→continuous casting→slab heating→hot rolling→pickling+cold rolling→continuous annealing→(pre-coating)→finishing packaging→blanking→heating→die stamping and quenching. There is a shortage of long production process and high cost. For some anti-collision or load-bearing parts, multiple parts combined with members

are used to improve the anti-collision and load-carrying capacity, which leads to greatly increased raw material cost and processing cost.

With the development of iron and steel industry, a medium and thin slab casting and direct rolling process has been greatly developed. The medium and thin slab casting and direct rolling process can directly produce steel sheet and strip with a nominal thickness of more than 0.2 mm-2.0 mm. Some thin-specification parts only adopting cold-rolled high-strength steels or members composed of multiple parts for strengthening have been gradually replaced by direct rolling ultra-high-strength steel sheet using a slab casting and direct rolling process. For example, a Patent Application No. CN 102965573A has developed a high-strength steel for engineering structures with a yield strength ( $R_{eL}$ ) of 700 MPa or more and a tensile strength ( $R_m$ ) of 750 MPa or more. The steel sheet has the chemical composition of: C: 0.15-0.25%, Si: 0.10%, Mn: 1.00-1.80%, P: 0.020%, S: 0.010%, Ti: 0.09-0.20%, Als: 0.02-0.08%, N: 0.008%, and a balance of Fe and inevitable impurities, in terms of % by mass. The invention steel sheet can be produced by a production method including: smelting and continuous casting into a slab, soaking, and controlling the soaking temperature to be 1200-1300° C. and a soaking time to be 20-60 min; hot rolling, and controlling a rolling temperature to be not lower than 1200° C. and a finishing rolling temperature to be 870-930° C.; performing laminar cooling, cooling to a cooling temperature at a cooling speed of not lower than 20° C./s.; and performing coiling, and controlling the cooling temperature to be 580-650° C. A Patent No. CN 103658178A invents a short-flow method for producing a high-strength thin strip steel. The invented strip steel has a yield strength ( $R_{eL}$ ) greater than or equal to 550 MPa and a tensile strength ( $R_m$ ) greater than or equal to 600 MPa. The strip steel includes following chemical components by mass percent: C: 0.02-0.15%, Si: 0.20-0.6%, Mn: 0.2-1.50%, P: 0.02-0.3%, S: 0.006%, Cr: 0.40-0.8%, Ni: 0.08-0.40%, Cu: 0.3-0.80%, Nb: 0.010-0.025%, Ti: 0.01-0.03%, Al: 0.01-0.06%, Re: 0.02-0.25%, and a balance of Fe and inevitable impurities. After smelting, a casting strip with a thickness of 1.0-2.0 mm is cast at a casting speed of 60-150 m/min; rolling is performed, and a finishing rolling temperature is controlled to be 850-1000° C.; atomization cooling is adopted at a cooling speed of 50-100° C./s., coiling is performed, and a coiling temperature is controlled to be 520-660° C. The tensile strength of the above two documents is very low, which cannot meet a demand of a high-end automobile body for ultra-high strength of 1900 MPa or more.

**SUMMARY OF THE INVENTION**

The present invention is directed to a press hardening steel having a tensile strength of 1900 MPa or more and a production method thereof, which can meet requirements of automobile design for ultra-high-strength and can also successfully complete complex deformation with no springback after deformation and high dimensional accuracy of parts, so as to overcome the shortcomings in the prior art that a strength level is low and the demands of a user for high-strength parts cannot be met.

Measures for achieving the foregoing objectives are taken as follows.

A press hardening steel is rolled directly from a thin slab and has a tensile strength of 1900 MPa or more. The press hardening steel sheet has the chemical composition of: C: 0.31-0.40%, Si: 0.36-0.44%, Mn: 1.6-2.0%, P: 0.006%, S: 0.004%, Als: 0.015-0.060%, Cr: 0.36-0.49%, Ti: 0.036-

0.045% or Nb: 0.036-0.045% or V: 0.036-0.045%, or a mixture of any two or more of the above in any proportion, B: 0.004-0.005%, Mo: 0.26-0.35%, N≤0.005%, and a balance of Fe and inevitable impurities, in terms of % by mass. A quenched microstructure is a full lath martensite. Mechanical properties are as follows: yield strength ≥1300 MPa, tensile strength ≥1900 MPa, and elongation A<sub>80 mm</sub>≥5%.

A method for producing the press hardening steel rolled directly from the thin slab casting and direct rolling and having the tensile strength of 1900 MPa or more is characterized by including the following steps:

1) Hot melt desulphurizing, and controlling S≤0.002%, an exposed surface of the molten iron after slagging off being not lower than 96%.

2) Performing conventional electric furnace or converter smelting, and conventional refining.

3) Performing continuous casting, and controlling a degree of superheat of tundish molten steel to be in the temperature of 15-30° C., a thickness of a slab to be 48-52 mm, and the casting speed to be 4.0-7.0 m/min.

4) Performing descaling treatment before the slab enters a soaking furnace, and controlling a pressure of descaling water to be 300-400 bar.

5) Performing conventional soaking on the slab, and controlling inside of the soaking furnace in a weak oxidizing atmosphere, i.e. a residual oxygen content in the furnace being 0.5-5.0%.

6) Heating the slab, and controlling a temperature of the slab entering the furnace to be 850-1050° C. and a tapping temperature of the slab leaving the furnace to be 1210-1230° C.

7) Performing high-pressure water descaling before entering a rolling mill, and controlling the pressure of the descaling water to be 280-420 bar.

8) Hot rolling, controlling a first pass reduction rate to be 52-63%, a second pass reduction rate to be 50-60% and a final pass reduction rate to be 10-16%, controlling a rolling speed to be 8-12 m/s, performing medium-pressure water descaling between a first pass and a second pass under the pressure of the descaling water of 200-280 bar, and controlling a finishing rolling temperature to be 870-910° C.

9) Cooling to a coiling temperature in a manner of laminar cooling, water curtain cooling or intensified cooling.

10) Performing coiling, and controlling the cooling temperature to be 605-635° C.

11) Performing austenitizing after uncoiling and blanking, controlling an austenitizing temperature to be 850-920° C., and holding for 3-5 min.

12) Die punching and deforming, and keeping the pressure for 10-20 s in a die.

13) Performing quenching, controlling a quenching cooling speed to be 20-40° C./s, and then naturally cooling to a room temperature.

The method is characterized in that the rolling process of the medium and thin slab is carried out in a short-process production line in any one of rolling mill arrangement forms such as a 6F production line or a 1R+6F production line, or a 2R+6F production line, or a 7F production line, or a 3R+4F production line, or 2R+5F production line, or a 1R+5F production line.

Mechanism of Each Element and Main Process in the Present Invention

C: Carbon is a strong solution strengthening element, which plays a decisive role in the acquisition of ultra-high strength. The carbon content has a great influence on the microstructures and properties of the final product, but the

content is too high, and it is easy to form a large amount of pearlite or bainite or martensite in the cooling process after finish rolling. The higher the content, the higher the strength, which results in a decrease in plasticity and difficulty in blanking before forming. Therefore, under the premise of ensuring heat treatment strengthening, the carbon content should not be too high. Therefore, the content is limited to a range of 0.31% to 0.40%.

Si: Silicon has a strong solution strengthening effect, which can improve the strength of steel. Furthermore, silicon can improve a hardenability of steel and reduce a volume change of austenite transforms into martensite, thus effectively controlling the production of quenching cracks. During low temperature tempering, a diffusion of carbon can be hindered, and the decomposition of martensite and the aggregation and growth of carbide are delayed, so that a hardness of steel decreases slowly during tempering, which significantly improves a tempering stability and strength of steel. Therefore, the content is limited to a range of 0.36% to 0.44%.

Mn: Manganese acts as a solution strengthening agent, and furthermore, it can remove FeO in steel and significantly improve the quality of steel. It can also form MnS with a high melting point with sulphide. In thermal processing, MnS has sufficient plasticity to prevent steel from hot shortness, reduce the harmful effects of sulphur, and improve the hot workability of steel. Manganese can reduce a phase change driving force, make a "C" curve shift to the right, improve the hardenability of steel, enlarge a γ phase region, and reduce the M<sub>3</sub> point of steel, so it can be ensured that martensite is obtained at a suitable cooling speed. Therefore, the content is limited to a range of 1.6% to 2.0%.

Cr: Chromium can reduce the phase transformation driving force and also reduce the nucleation growth of carbides during phase transformation, so the hardenability of steel is improved. In addition, chromium can improve the tempering stability of steel. Therefore, the content is limited to a range of 0.36% to 0.49%.

B: Boron is an element that strongly enhances hardenability. The addition of trace amounts of boron to steel can significantly improve the hardenability of the steel. However, the content is lower than 0.0005%, or higher than 0.0050%, and the effect on improving hardenability is not obvious. Therefore, in order to consider the actual production and hardenability effects, the content is limited to a range of 0.004% to 0.005%.

Als: It deoxidizes in steel, it should be ensured that there is a certain amount of acid-soluble aluminium in the steel, otherwise it will not exert its effect, but too much aluminium will cause aluminium-based inclusions in the steel, which is not conducive to steel smelting and casting. Furthermore, the addition of an appropriate amount of aluminium in steel can eliminate the adverse effects of nitrogen and oxygen atoms on the properties of the steel. Therefore, the content is limited to a range of 0.015% to 0.060%.

P: Phosphorus is a harmful element in steel, which is liable to cause segregation in a centre of a slab. In the subsequent hot continuous rolling heating process, it tends to be segregated to a grain boundary, so that a brittleness of steel is significantly increased. Furthermore, based on cost considerations and without affecting the properties of the steel, the content is controlled to be 0.006% or less.

S: Sulphur is a very harmful element. Sulphur in steel is often present in the form of sulphides of manganese. This sulphide inclusion can deteriorate a toughness of the steel and cause anisotropy of properties. Therefore, it is necessary to control the sulphur content in the steel as low as possible.

The sulphur content in the steel is controlled to be 0.004% or less based on consideration of manufacturing cost.

N: Nitrogen can be combined with titanium to form titanium nitride in titanium-added steel. This second phase precipitated at high temperature is beneficial for strengthening a matrix and improving a weldability of a steel plate. However, the nitrogen content is higher than 0.005%, and a solubility product of nitrogen and titanium is higher. At high temperature, a coarse titanium nitride is formed in the steel, which seriously damages the plasticity and toughness of the steel. In addition, the higher nitrogen content will increase the amount of micro-alloying elements required to stabilize the nitrogen element, thereby increasing the cost. Therefore, the content is controlled to be less than 0.005%.

Ti: Titanium is a strong C and N compound forming element. The purpose of adding Ti to steel is to fix the N element in the steel, but the excess Ti will combine with C to reduce the hardness and strength of martensite after quenching of the test steel. In addition, the addition of titanium contributes to the hardenability of steel. Therefore, the content is limited to a range of 0.036% to 0.045%.

Nb, V: Niobium and vanadium are also strong C and N compound forming elements, which can refine austenite grains. A small amount of niobium or vanadium can be added into steel to form a certain amount of niobium carbon and nitride, so that growth of the austenite grain is hindered, and therefore, a size of a martensite lath after quenching is small, and the strength of the steel is greatly improved. Therefore, the content is controlled between 0.036% and 0.045%.

Mo: Molybdenum can significantly improve the hardenability of steel, and a stacking fault energy of molybdenum is high. The addition of the molybdenum into steel can improve the low temperature plasticity and toughness of the steel. Therefore, the content is controlled between 0.26% and 0.35%.

The reason why the present invention adopts three times of descaling in the whole production process is that mill scale on a surface of a strip steel can be removed maximally by controlling the descaling pass and the appropriate descaling water pressure, thereby ensuring that the strip steel has a good surface quality. In addition, the microstructure uniformity and property stability of the strip steel can be realized by controlling the first pass reduction rate, the second pass reduction rate and the final pass reduction rate.

Compared with the prior art, the present invention is high in strength, has a short manufacturing process and good product surface quality, and the accuracy of thickness may be controlled within  $\pm 0.03$  mm, thus greatly reducing energy consumption; in addition, compared with existing products directly rolled through medium and thin slabs, the strength is much higher than that of the existing products, which is of great significance for reducing the weight of automobiles.

#### BRIEF DESCRIPTION OF THE DRAWINGS

FIG. 1 is a microstructure of a product according to the present invention.

#### DESCRIPTION OF THE EMBODIMENTS

The present invention is described in detail below.

Table 1 is a list of chemical component values of various embodiments and comparative examples of the present invention.

Table 2 is a list of main process parameter of various embodiments and comparative examples of the present invention.

5 Table 3 is a list of property detection cases of various embodiments and comparative examples of the present invention.

In various embodiments of the present invention, production is performed according to following process:

10 1) Hot melt desulphurize molten iron, and control S $\leq$ 0.002%, an exposed surface of the molten iron after slagging off being not lower than 96%.

15 2) Perform conventional electric furnace or converter smelting, and conventional refining.

20 3) Perform continuous casting, and control a degree of superheat of tundish molten steel to be in the temperature of 15-30° C., a thickness of a slab to be 48-52 mm, and the casting speed to be 4.0-7.0 m/min.

25 4) Perform descaling treatment before the slab enters a soaking furnace, and control a pressure of descaling water to be 300-400 bar.

30 5) Perform conventional soaking on the slab, and control inside of the soaking furnace in a weak oxidizing atmosphere, i.e. a residual oxygen content in the furnace being 0.5-5.0%.

35 6) Heat the slab, and control a temperature of the slab entering the furnace to be 850-1050° C. and a tapping temperature of the slab leaving the furnace to be 1210-1230° C.

40 7) Perform high-pressure water descaling before entering a rolling mill, and control the pressure of the descaling water to be 280-420 bar.

45 8) Perform hot rolling, control a first pass reduction rate to be 52-63%, a second pass reduction rate to be 50-60% and a final pass reduction rate to be 10-16%, control a rolling speed to be 8-12 m/s, perform medium-pressure water descaling between a first pass and a second pass under the pressure of the descaling water of 200-280 bar, and control a finishing rolling temperature to be 870-910° C.

50 9) Cool to a coiling temperature in a manner of laminar cooling, water curtain cooling or intensified cooling.

10) Perform coiling, and control a coiling temperature to be 605-635° C.

55 11) Perform austenitizing after uncoiling and blanking, control an austenitizing temperature to be 850-920° C., and hold for 3-5 min.

12) Perform die punching and deforming, and keep a pressure for 10-20 s in a die.

60 13) Perform quenching, control a quenching cooling speed to be 20-40° C./s, and then naturally cool to the room temperature.

The rolling process of the thin slab is carried out in a short-process production line in any one of rolling mill arrangement forms such as a 6F production line or a 1R+6F production line, or a 2R+6F production line, or a 7F production line, or a 3R+4F production line, or 2R+5F production line, or a 1R+5F production line.

TABLE 1

| Embodiment | C    | Si   | Mn   | P     | S     | Als   | Cr   | Ti    | Nb    | V     | Mo   | B      | N     |
|------------|------|------|------|-------|-------|-------|------|-------|-------|-------|------|--------|-------|
| 1          | 0.38 | 0.42 | 1.9  | 0.004 | 0.004 | 0.027 | 0.38 | 0.045 | —     | —     | 0.27 | 0.0042 | 0.003 |
| 2          | 0.36 | 0.43 | 1.7  | 0.005 | 0.002 | 0.036 | 0.49 | 0.042 | 0.036 | —     | 0.26 | 0.0045 | 0.002 |
| 3          | 0.40 | 0.36 | 1.6  | 0.005 | 0.003 | 0.029 | 0.47 | —     | 0.045 | —     | 0.30 | 0.0040 | 0.004 |
| 4          | 0.32 | 0.39 | 1.8  | 0.004 | 0.004 | 0.060 | 0.48 | —     | 0.044 | 0.041 | 0.29 | 0.0048 | 0.005 |
| 5          | 0.35 | 0.40 | 1.95 | 0.006 | 0.001 | 0.015 | 0.36 | 0.036 | —     | —     | 0.35 | 0.0050 | 0.004 |
| 6          | 0.31 | 0.44 | 2.0  | 0.003 | 0.002 | 0.055 | 0.45 | —     | —     | 0.045 | 0.34 | 0.0049 | 0.002 |
| 7          | 0.39 | 0.38 | 1.75 | 0.005 | 0.002 | 0.043 | 0.42 | 0.038 | —     | 0.036 | 0.32 | 0.0041 | 0.003 |

TABLE 2

| List of main process parameter values of various embodiments and comparative examples of the present invention |                                       |                          |                                 |                          |                                |                              |                                |                               |
|----------------------------------------------------------------------------------------------------------------|---------------------------------------|--------------------------|---------------------------------|--------------------------|--------------------------------|------------------------------|--------------------------------|-------------------------------|
| Embodiment                                                                                                     | Temperature of slab into furnace ° C. | Tapping temperature ° C. | Finish rolling temperature ° C. | Cooling temperature ° C. | Austenitizing temperature ° C. | Temperature holding time min | Quenching cooling speed ° C./s | Pressure keeping time in dies |
| 1                                                                                                              | 1036-1050                             | 1210-1222                | 880-900                         | 616-630                  | 920                            | 3                            | 33                             | 14                            |
| 2                                                                                                              | 954-969                               | 1220-1230                | 896-910                         | 623-635                  | 900                            | 4                            | 29                             | 17                            |
| 3                                                                                                              | 880-891                               | 1212-1225                | 870-889                         | 605-617                  | 910                            | 3                            | 38                             | 18                            |
| 4                                                                                                              | 995-1008                              | 1216-1229                | 882-895                         | 608-623                  | 880                            | 4                            | 20                             | 10                            |
| 5                                                                                                              | 850-863                               | 1211-1223                | 889-902                         | 622-634                  | 850                            | 5                            | 24                             | 16                            |
| 6                                                                                                              | 1019-1030                             | 1219-1230                | 883-898                         | 612-627                  | 890                            | 3                            | 22                             | 12                            |
| 7                                                                                                              | 875-887                               | 1215-1227                | 875-887                         | 615-632                  | 860                            | 5                            | 40                             | 20                            |

TABLE 3

| List of mechanical property cases of various embodiments and comparative examples of the present invention |              |                                      |                                     |                                 |
|------------------------------------------------------------------------------------------------------------|--------------|--------------------------------------|-------------------------------------|---------------------------------|
| Component                                                                                                  | Thickness mm | Yield strength R <sub>p0.2</sub> MPa | Tensile strength R <sub>m</sub> MPa | Elongation A <sub>80 mm</sub> % |
| 1                                                                                                          | 0.8          | 1420                                 | 2050                                | 5.2                             |
| 2                                                                                                          | 1.5          | 1390                                 | 1970                                | 5.8                             |
| 3                                                                                                          | 1.2          | 1410                                 | 1985                                | 5.4                             |
| 4                                                                                                          | 2.0          | 1330                                 | 1920                                | 6.2                             |
| 5                                                                                                          | 1.8          | 1350                                 | 1950                                | 5.9                             |
| 6                                                                                                          | 1.0          | 1400                                 | 2010                                | 5.4                             |
| 7                                                                                                          | 0.9          | 1395                                 | 2000                                | 5.5                             |

As can be seen from Table 3, a short process for direct rolling from a thin slab makes the strength of the inventive steel up to 2100 MPa, which can achieve the purpose of replacing cold forming with press hardening and is of great significance for promoting the development of lightweight automobiles.

The present specific implementation is merely exemplary and does not limit the implementation of the technical solutions of the present invention.

What is claimed is:

1. A method for producing a press hardening steel, the press hardening steel having a tensile strength of 1900 MPa or more, and comprising following components by weight percent: C: 0.31-0.40%, Si: 0.36-0.44%, Mn: 1.6-2.0%, P≤0.006%, S≤0.004%, Als: 0.015-0.060%, Cr: 0.36-0.49%, Ti: 0.036-0.045% or Nb: 0.036-0.045% or V: 0.036-0.045% or a mixture of any two or more of the above in any proportion, B: 0.004-0.005%, Mo: 0.26-0.35%, and N≤0.005%, and a balance of Fe and inevitable impurities, the method comprising following steps:

- 35 1) desulphurizing molten iron, and controlling S to be smaller or equal to 0.002%, an exposed surface of the molten iron after slagging off being not lower than 96%;
- 2) performing electric furnace or converter smelting, and refining;
- 3) performing continuous casting, and controlling a degree of superheat of tundish molten steel to be 15° C. to 30° C., a thickness of a slab to be 48 mm to 52 mm, and a casting speed to be 4.0 m/min to 7.0 m/min;
- 4) performing descaling treatment before the slab enters a soaking furnace, and controlling a pressure of descaling water to be 300 bar to 400 bar;
- 5) performing soaking on the slab, and controlling inside of a soaking furnace in a weak oxidizing atmosphere in which the soaking furnace has an atmosphere in which the oxygen content is 0.5% to 5.0%;
- 40 6) heating the slab, and controlling a temperature of the slab entering the furnace to be 850° C. to 1050° C. and a tapping temperature of the slab leaving the furnace to be 1210° C. to 1230° C.;
- 7) performing high-pressure water descaling before entering a rolling mill, and controlling the pressure of the descaling water to be 280 bar to 420 bar;
- 45 8) hot rolling, controlling a first pass reduction rate to be 52% to 63%, a second pass reduction rate to be 50% to 60% and a final pass reduction rate to be 10% to 16%, controlling a rolling speed to be 8 m/s to 12 m/s, performing medium-pressure water descaling between a first pass and a second pass under the pressure of the descaling water of 200 bar to 280 bar, and controlling a finishing rolling temperature to be 870° C. to 910° C.;
- 9) cooling to a cooling temperature in a manner of laminar cooling, water curtain cooling or intensified cooling;

- 10) performing coiling, and controlling a coiling temperature to be 605° C. to 635° C.;
- 11) performing austenitizing after uncoiling and blanking, controlling an austenitizing temperature to be 910° C. to 920° C., and holding for 3 minutes to 4 minutes; 5
- 12) performing die stamping forming, and keeping a pressure for 10 seconds to 20 seconds in a die; and
- 13) performing quenching, controlling a quenching cooling speed to be 20° C./s to 24° C./s, and then naturally cooling to room temperature. 10

2. The method for producing the press hardening steel according to claim 1, wherein: the hot rolling of the slab is carried out in a short-process production line in any one of rolling mill arrangement forms a 6 finishing mills production line or a 1 roughing mill+6 finishing mills production line, 15 or a 2 roughing mills+6 finishing mills production line, or a 7 finishing mills production line, or a 3 roughing mills+4 finishing mills production line, or 2 roughing mills+5 finishing mills production line, or a 1 roughing mill+5 finishing mills production line. 20

\* \* \* \* \*